

Feb. 4, 1969

R. C. TABER ET AL

3,425,833

MORDANTS FOR BLEACHABLE FILTER LAYERS

Filed Aug. 16, 1965

FIG. 1



FIG. 2



FIG. 3



ROBERT C. TABER  
DUGALD A. BROOKS  
INVENTORS

BY *R. Frank Smith*  
*Ray Carter Swenson*

ATTORNEY & AGENT

1

3,425,833

**MORDANTS FOR BLEACHABLE FILTER LAYERS**  
 Robert C. Taber and Dugald A. Brooks, Rochester, N.Y.,  
 assignors to Eastman Kodak Company, Rochester,  
 N.Y., a corporation of New Jersey

Filed Aug. 16, 1965, Ser. No. 479,720

 U.S. Cl. 96—84  
 Int. Cl. G03c 1/84

12 Claims

This invention relates to certain bulky, i.e., relatively high molecular weight, quaternary nitrogen heterocyclic compounds containing a phenolic group which function as "alkali-release" mordants, to photographic materials and more particularly to photographic elements containing these compounds in light-screening and light-absorbing layers, and to methods for their preparation.

The use of organic dye containing light-filter and light-absorbing layers in photographic elements is well known, as is the use of mordants which form substantially insoluble salts or otherwise react with water-soluble dyes, to render the dyes non-diffusing. Such dye-mordant light-screening salt may be in a layer overlying a light-sensitive emulsion or overlying two or more light-sensitive emulsions; or it may be in a light-sensitive emulsion for the purpose of modifying a light record in such emulsion or for protecting an overlying light-sensitive emulsion or emulsions from the action of light of wavelengths absorbed by such light-screening substance, or it may be in a layer not containing a light-sensitive substance but arranged between two light-sensitive emulsions; or it may be in a layer serving as a backing on an element having one or more light-sensitive emulsions (for example, to reduce halation).

In particular, light-screening substances are often required (a) in overcoatings upon photographic elements to protect the light-sensitive emulsion or emulsions from the action of light which it is not desired to record, (b) in layers arranged between differentially color sensitized emulsions, e.g., to protect red- and green-sensitive emulsions from the action of blue light, and (c) in backings forming the so-called anti-halation layers on either side of a transparent support carrying the light-sensitive emulsion or emulsions.

In most cases and especially where the element contains a color sensitized emulsion or color sensitized emulsions, it is particularly desirable to employ light-screening substances which do not affect the general sensitivity or the color sensitivity of light-sensitive emulsions with which they may come into contact. It is also particularly desirable to employ light-screening substances which do not substantially diffuse from the layers or coatings in which they are incorporated, either during the manufacture of the element or on storing it or in photographically processing it. Finally it is generally necessary to employ light-screening substances which can readily be rendered ineffective, i.e., decolorized or destroyed and removed prior to or during or after photographic processing. For many purposes it is particularly convenient to employ light-screening substances which are rendered ineffective by one of the photographic baths employed in processing the element after exposure, such as a photographic developing bath or fixing bath.

Numerous substances have been proposed as mordants to prepare the dye-mordant salts used as light-screening and light-absorbing materials for the purposes indicated above. Among the proposed mordants are relatively high molecular weight compounds having ionic charges opposite to those of the particular light-absorbing dye. For example, the dye employed might be an acid dye, in which case the mordant would be a cationic. Typical of such proposed mordants are, for example, derived polymers such as the basic reaction products of polyvinylsulfonates and C-aminopyridines as described in D. D. Reynolds et

2

al., U.S. Patents 2,701,243 and 2,768,078, granted Feb. 1, 1955, and Oct. 23, 1956, respectively. While polymeric mordants such as illustrated by the above-mentioned patents have the advantage of bulky molecules and do function to fix acid dyes in photographic layers, within their particular limitations, they have not been found entirely satisfactory in many applications primarily because these polymeric mordants on alkaline development and release of the dye, still retain their mordanting property and, accordingly, not only tend to retain some residual dye as evidences by background stain or coloration in the layers, but more importantly retain, i.e., fix an appreciable amount of thiosulfate ion in the subsequent hypo processing used to remove unexposed silver halide. 15 This results in relatively poor quality and poor keeping 20 stability of the produced images. In view of this, it would be very desirable to have an effective mordant available that is free from such disadvantages.

We have now found that certain bulky quaternary 25 nitrogen heterocyclic compounds containing phenolic groups are especially useful as precipitants and mordants for acid dyes in photographic layers, and that these compounds satisfactorily overcome the above-mentioned shortcomings of heretofore known mordants for this purpose. Thus, when incorporated in photographic layers, they function effectively as "alkali-release" mordants without retention of any residual dye or deleterious amounts of thiosulfate ion in the layers on processing, and the 30 produced images are of very good quality and of outstanding keeping properties. These mordants are soluble in aqueous solutions, for example, dilute solutions of acids such as acetic, butyric, lauric, etc. acids. Furthermore, they readily form substantially non-diffusible salts with water-soluble dyes, and these are all compatible with 35 various hydrophilic materials such as gelatin. They are compounds of definite constitution and, in general, have molecular weights of about at least 300.

It is, accordingly, an object of the invention to provide 40 a photographic element having one or more layers containing at least one of the bulky nitrogen heterocyclic compounds or salts of the invention described above. Another object is to provide a backing layer containing at least one of these salts. Another object is to provide a light filter layer containing at least one of the above 45 salts; which layer may be coated between two or more silver halide emulsion layers in a multilayer element. Another object is to provide an imbibition blank containing at least one of the above salts. Another object is to provide a light-sensitive gelatin-silver halide layer containing 50 at least one of the above salts. Another object is to provide overcoating layers for photographic elements which contain at least one of the above salts. Another object is to provide a process for preparing the bulky 55 quaternary nitrogen heterocyclic compounds and salts thereof. Other objects will become apparent from consideration of the description and the examples.

The phenolic group containing bulky quaternary heterocyclic compounds that are useful as "alkali-release" mordants include those represented by the following 60 general formulas:



65 70 wherein *d*, *m* and *n* represent an integer of from 1 to 2, *R* represents the hydrogen atom, an alkyl group (e.g., methyl, ethyl, propyl, isopropyl, butyl, hexyl, dodecyl,

etc.), an aryl group (e.g., phenyl, tolyl, naphthyl, a phenolic group or ring such as p-hydroxyphenyl, 4-hydroxy-3,5-dibromophenyl, 2-hydroxy-5-octylphenyl, 5-hydroxynaphthyl, etc.), R<sub>1</sub> represents an alkyl group (e.g., methyl, ethyl, propyl, isopropyl, butyl, hexyl, dodecyl, etc.), an aryl group (e.g., phenyl, tolyl, naphthyl, a phenolic group or ring such as p-hydroxyphenyl, 4-hydroxy-3,5-dibromophenyl, 2-hydroxy-5-octylphenyl, 4-hydroxynaphthyl, etc.), R<sub>2</sub> and R<sub>3</sub> each represents an alkyl group (e.g., methyl, ethyl, propyl, isopropyl, butyl, hexyl, dodecyl, etc.), an aryl group (e.g., phenyl, tolyl, naphthyl, etc.), or an aralkyl group (e.g., benzyl, phenethyl, etc.), R<sub>2</sub> and R<sub>3</sub> together represent a divalent straight or branched chain alkylene group having from 4 to 5 carbon atoms in the chain (e.g., tetramethylene, pentamethylene, 4-methylpentamethylene, etc.), X represents an acid anion (e.g., chloride, bromide, iodide, thiocyanate, sulfamate, perchlorate, methyl sulfate, ethyl sulfate, p-toluenesulfonate, etc.), B represents the group CH=CH, the group (CH=CH)<sub>2</sub>, the group (CH=CH)<sub>3</sub>, or the p-phenylene group, and Z represents the nonmetallic atoms required to complete a heterocyclic nucleus having from 5-6 members in the heterocyclic ring, such as a thiazole nucleus

(e.g., thiazole,  
4-methylthiazole,  
4-phenylthiazole,  
4'-p-hydroxyphenyl)-thiazole,  
5-methylthiazole,  
5-phenylthiazole,  
5-(o-hydroxyphenyl)-thiazole,  
4,5-dimethylthiazole,  
4,5-diphenylthiazole,  
4-(2-thienyl)thiazole, etc.),  
a benzothiazole nucleus  
(e.g., benzothiazole,  
4-hydroxybenzothiazole,  
4-chlorobenzothiazole,  
5-chlorobenzothiazole,  
6-chlorobenzothiazole,  
7-chlorobenzothiazole,  
4-methylbenzothiazole,  
5-methylbenzothiazole,  
6-methylbenzothiazole,  
5-bromobenzothiazole,  
6-bromobenzothiazole,  
4-phenylbenzothiazole,  
5-phenylbenzothiazole,  
4-methoxybenzothiazole,  
5-methoxybenzothiazole,  
6-methoxybenzothiazole,  
5-iodobenzothiazole,  
6-iodobenzothiazole,  
4-ethoxybenzothiazole,  
5-ethoxybenzothiazole,  
tetrahydrobenzothiazole,  
5,6-dimethoxybenzothiazole,  
5,6-dioxymethylenebenzothiazole,  
5-hydroxybenzothiazole,  
6-hydroxybenzothiazole, etc.),  
a naphthothiazole nucleus  
(e.g.,  $\alpha$ -naphthothiazole,  
 $\beta$ -naphthothiazole,  
5-methoxy- $\beta$ -naphthothiazole,  
5-ethoxy- $\beta$ -naphthothiazole,  
7-methoxy- $\alpha$ -naphthothiazole,  
8-methoxy- $\alpha$ -naphthothiazole,  
5-hydroxy- $\beta$ -naphthothiazole,  
7-hydroxy- $\alpha$ -naphthothiazole, etc.),  
a thianaphtheno-7',6',4,5-thiazole nucleus  
(e.g., 4-methoxythianaphtheno-7',6',4,5-thiazole, etc.),  
an oxazole nucleus  
(e.g., 4-methyloxazole,  
5-methyloxazole,  
4-phenyloxazole,

4-(p-hydroxyphenyl)oxazole,  
4,5-diphenyloxazole,  
4-ethyloxazole,  
4,5-dimethyloxazole,  
5-phenyloxazole,  
5-(m-hydroxyphenyl)oxazole, etc.),  
a benzoxazole nucleus  
(e.g., benzoxazole,  
5-chlorobenzoxazole,  
5-methylbenzoxazole,  
5-phenylbenzoxazole,  
6-methylbenzoxazole,  
5,6-dimethylbenzoxazole,  
4,6-dimethylbenzoxazole,  
5-methoxybenzoxazole,  
5-ethoxybenzoxazole,  
6-chlorobenzoxazole,  
6-methoxybenzoxazole,  
5-hydroxybenzoxazole,  
6-hydroxybenzoxazole, etc.),  
a naphthoxazole nucleus  
(e.g.,  $\alpha$ -naphthoxazole,  
 $\beta$ , $\beta$ -naphthoxazole,  
 $\beta$ -naphthoxazole,  
6-hydroxy- $\beta$ -naphthoxazole, etc.),  
a selenazole nucleus  
(e.g., 4-methylselenazole,  
4-phenylselenazole,  
4-(p-hydroxyphenyl) selenazole, etc.),  
a benzoselenazole nucleus  
(e.g., benzoselenazole,  
5-chlorobenzoselenazole,  
5-methoxybenzoselenazole,  
5-hydroxybenzoselenazole,  
tetrahydrobenzoselenazole, etc.),  
a naphthoselenazole nucleus  
(e.g.,  $\alpha$ -naphthoselenazole,  
 $\beta$ , $\beta$ -naphthoselenazole,  
 $\beta$ -naphthoselenazole,  
7-hydroxy- $\beta$ -naphthoselenazole, etc.),  
a thiazoline nucleus  
(e.g., thiazoline,  
4-methylthiazoline,  
4-(p-hydroxyphenyl)thiazoline, etc.),  
a quinoline nucleus  
(e.g., quinoline,  
3-methylquinoline,  
5-methylquinoline,  
7-methylquinoline,  
8-methylquinoline,  
6-chloroquinoline,  
8-chloroquinoline,  
6-methoxyquinoline,  
6-ethoxyquinoline,  
6-hydroxyquinoline,  
8-hydroxyquinoline, etc.),  
an isoquinoline nucleus  
(e.g., isoquinoline,  
3-methylisoquinoline,  
5-methylisoquinoline,  
6-chloroisoquinoline,  
6-methoxyisoquinoline,  
8-hydroxyisoquinoline, etc.),  
a 3,3-dialkylindolenine nucleus  
(e.g., 3,3-dimethylindolenine,  
5-hydroxy-3,3-dimethylindolenine,  
3,3,5-trimethylindolenine,  
3,3,7-trimethylindolenine, etc.),  
a pyridine nucleus  
(e.g., pyridine,  
4-methylpyridine,  
6-methylpyridine,  
4,6-dimethylpyridine,  
4-butylpyridine,  
4-decylpyridine,  
4-octadecylpyridine,

4,6-dibutylpyridine,  
4-benzylpyridine,  
6-benzylpyridine,  
4-phenylpyridine,  
4-(p-hydroxyphenyl)pyridine,  
4,6-diphenylpyridine,  
4,6-dinaphthylpyridine,  
4-(2-thienyl)pyridine,  
6-(2-thienyl)pyridine,  
4,6-di(2-thienyl)pyridine,  
4-(2-pyrryl)pyridine,  
4-(2-indolyl)pyridine,  
4-(3-indolyl)pyridine,  
4-(3-pyridyl)pyridine,  
4-(4-pyridyl)pyridine,  
4,6-di(2-pyrryl)pyridine,  
4-chloropyridine,  
4-bromopyridine,  
4,6-dichloropyridine,  
4-chloro-6-bromopyridine,  
4-phenoxyppyridine,  
4-alkoxypyridines,  
6-alkoxypyridines,  
4,6-dialkoxypyridine,  
4-(2-furyl)pyridine, etc.),  
an imidazole nucleus  
(e.g., imidazole,  
1-alkylimidazole,  
1-alkyl-4-phenylimidazole,  
4-(p-hydroxyphenyl)imidazole,  
1-alkyl-4,5-dimethylimidazole, etc.),  
a benzimidazole nucleus  
(e.g., benzimidazole,  
5-hydroxybenzimidazole,  
1-alkylbenzimidazole,  
1-aryl-5,6-dichlorobenzimidazole, etc.),  
a naphthimidazole nucleus  
(e.g., 1-alkyl- $\alpha$ -naphthimidazole,  
1-aryl- $\beta$ -naphthimidazole,  
1-alkyl-5-methoxy- $\alpha$ -naphthimidazole,  
1-alkyl-6-hydroxy- $\beta$ -naphthimidazole, etc.),  
a thiadiazole nucleus  
(e.g., 1,2,4-thiadiazole),  
an oxadiazole nucleus  
(e.g., 1,2,4-oxadiazole,  
1,3,4-oxadiazole,  
5-(p-hydroxyphenyl)-1,2,4-oxadiazole, etc.),  
a 1 or 4 alkyl or aryl-1,2,4-triazole nucleus  
(e.g., 1-methyl-1,2,4-triazole,  
1-butyl-1,2,4-triazole,  
5-(p-hydroxyphenyl)-1,2,4-triazole, etc.),  
a tetrazole nucleus  
(e.g., tetrazole,  
5-butyl-1,2,3,4-tetrazole,  
5-phenyl-1,2,3,4-tetrazole,  
5-(o-hydroxyphenyl)-1,2,3,4-tetrazole, etc.),

and the like nuclei. The components of Formulas I and II are so chosen as to give compounds having molecular weights in each instance of at least 300. They are further chosen so that at least one of the members represented by R, R<sub>1</sub> and Z in each instance contains a phenolic group or ring. It will be understood that the term "phenolic" as used herein also includes fused phenolic rings.

More particularly, the phenolic group or residue containing bulky quaternary nitrogen heterocyclic compounds of the invention that are especially suitable as "alkali-release" mordants in photographic layers include those represented by the following general formula:

III.



j represents an integer of from 1 to 3, d, and X are as 75

previously defined, R<sub>4</sub> and R<sub>0</sub> each represent a member, such as, the hydrogen atom, a halogen atom (e.g., chlorine or bromine), an alkyl group (e.g., methyl, ethyl, propyl, isopropyl, butyl, hexyl, dodecyl, octadecyl, benzyl, phenethyl, methoxymethyl, ethoxybutyl, isopropoxybutyl, butoxododecyl, etc.), an aryl group (e.g., phenyl, hydroxyphenyl, tolyl, naphthyl, etc.), an alkoxy group (e.g., methoxy, ethoxy, butoxy, etc.), an aryloxy group (e.g., phenoxy, tolyloxy, naphthoxy, etc.), or a heterocyclic nucleus (e.g., 2-thienyl, 2-pyrryl, 2-indolyl, 3-indolyl, 2-furyl, 3-pyridyl, 4-pyridyl, etc.). The R<sub>4</sub> and R<sub>0</sub> components and the values of d and j in Formula III above are so chosen as to give compounds having molecular weights in each instance of at least 300.

In accordance with the invention, we prepare the various salt compounds coming under Formula I above in a number of ways depending on the compounds to be prepared. For example, any of the pyridinium salts of Formula I can be readily prepared from the corresponding pyrylium salts by reaction with the appropriate amino-phenol intermediates as described hereinafter. Salts of most other heterocyclic bases where the phenolic residue is in the group on the nitrogen atom have to be prepared, for example, as illustrated in the following reaction where the R group contains a phenolic residue such as previously defined



and wherein d, n, B and X are as previously defined, and R<sub>5</sub> represents, for example, the hydrogen atom or an alkyl group. Those salts where the phenolic group is a substituent on the heterocyclic ring are conveniently prepared by a two step synthesis, for example, as illustrated in the following reaction:



wherein n, B, R, R<sub>1</sub> and X are as previously defined, and R<sub>6</sub> represents an alkyl group.

In place of the starting heterocyclic compounds in above reaction Formulas IV and V, there may be substituted any other of the heterocyclic compounds completed by Z in Formula I such as thiazoles, benzothiazoles, naphthothiazoles, oxazoles, benzoxazoles, naphthoxazoles, selenazoles, benzoselenazoles, naphthoselenazoles, thiazolines, quinolines, indolenines, imidazoles, benzimidazoles, naphthimidazoles, thiadiazoles, oxadiazoles, triazoles, tetrazoles, etc., to give the corresponding compounds of the invention defined by Formula I above.

Salts of the pyrrolidone and piperidine compounds com-

ing under Formula II above also require a two step synthesis, for example, as illustrated in the following reaction:

VI.



wherein R contains the phenolic residue such as defined previously, and d, n, R<sub>1</sub>, and X are as previously defined. It will be understood that one or more of the carbon atoms of the heterocyclic compound can be substituted with appropriate substituents, e.g., alkyl groups such as methyl, ethyl, etc.

To prepare the preferred pyridinium compounds of the invention coming under Formula III above, a pyrylium salt of the formula:

VII.



wherein j, R<sub>4</sub> and X are as previously defined, is reacted with a compound of the formula:

VIII.



wherein n, j, B, R<sub>4</sub>, and R<sub>0</sub> are as previously defined, in an inert organic solvent (e.g., benzene, toluene, etc.), in approximately equimolar proportions. Advantageously, the reaction is heated up to reflux temperature for a period of several minutes or more, at which time the solid product precipitates from solution. The product is collected on a filter funnel and can be used, if desired, without further purification. However, for greater purity, the precipitate can be washed with a nonsolvent such as benzene and dried. The above-described process is illustrated more specifically in Examples 1-3 hereinafter.

As previously mentioned, the above-defined mordants of the invention function as "alkali-release" mordants in photographic layers. Thus, under appropriate conditions of pH (i.e., alkaline conditions), they form a zwitterion with resultant internal charge compensation and at the same time lose their ability to act as mordants, with release and subsequent removal of the mordanted dye from the system. A major advantage of the above "alkali-release" mordants is, therefore, that the compounds do not retain either the previously mordanted dye or thiosulfate ion from the fixing, after processing, as do other compounds of similar mordanting ability, providing a neutral or mildly alkaline hypo bath is used.

The formation of the zwitterion upon treatment in alkali is illustrated below with the structure of above Formula IV.



wherein d, n, j, B, R<sub>4</sub>, R<sub>0</sub> and X are as previously defined.

The invention is further illustrated by the following examples describing the preparation and use of the mordanting compounds of the invention in photographic layers and elements.

5 Example 1.—1-m-hydroxyphenyl-2,4,6-triphenylpyridinium iodide



10 15 A one to one molar mixture of m-aminophenol and 2,4,6-triphenylpyrylium iodide in benzene was heated under reflux for two minutes at which time the solid product precipitated from solution. The product was then collected on a filter funnel and used without further purification. 20 This compound, at a ratio of 5 parts by weight to 1 part by weight of dye, mordanted the dye bis[3-methyl-1-p-sulfophenyl-2-pyrazolin-5-one-(4)]pentamethineoxonal in gelatin, with no bleeding upon washing in water. The 25 mordanted dye was bleached upon treatment of the coated gelatin layer (on a cellulose acetate film support) with a developer having the composition:

|                                |       |   |      |
|--------------------------------|-------|---|------|
| p-Methylaminophenol sulfate    | ----- | g | 4.5  |
| Sodium sulfite, desiccated     | ----- | g | 90.0 |
| 30 Hydroquinone                | ----- | g | 8.0  |
| Sodium carbonate, monohydrated | ----- | g | 52.5 |
| Potassium bromide              | ----- | g | 5.0  |
| Water to make 1 liter.         |       |   |      |

35 35 The bleaching was increased when the alkalinity of the developer was increased by the addition of sodium hydroxide. The residual yellow color was discharged by subsequent acidification of the gelatin layer. This was then treated with a fixing bath of the following composition:

|                            |       |    |       |
|----------------------------|-------|----|-------|
| 40 Sodium thiosulfate      | ----- | g  | 240.0 |
| Sodium sulfite, desiccated | ----- | g  | 15.0  |
| Acetic acid 28%            | ----- | cc | 48.0  |
| Boric acid, crystals       | ----- | g  | 7.5   |
| Potassium alum             | ----- | g  | 15.0  |
| 45 Water to make 1 liter.  |       |    |       |

Result.—Mordanted well. Bleached effectively in the developer. Retained no hypo from the fixing bath.

50 50 The above results for Example 1 were made for hand coatings on cellulose acetate film support, the melts for which were prepared as follows:

To 10 cc. of 10% photographic gelatin melted at 40° C. was added 30 or 50 mgs. of mordant dissolved in 10 cc. of the appropriate solvent. The pH of the solution was adjusted to 4.5-5.0 with glacial acetic acid. To this was then added 10 mgs. of bis[3-methyl-1-p-sulfophenyl-5-pyrazolone-(4)]pentamethineoxonal, dissolved in the appropriate solvent with vigorous stirring. The pH of the melt was then readjusted to 6.0±0.1 with 2.5 N NaOH, a coating aid added, the total volume adjusted to 32 cc. with distilled water and the melt coated and dried.

65 65 The bleed test consisted of immersing a portion of the hand coating in stagnant, distilled water at 75° F. for two minutes and inspecting for signs of dye bleeding out of the gel layer. If no bleeding was detected, the immersion was repeated for another two minute interval. Bleachability was determined by immersing a portion of the hand coating in the developer for two minutes and observing the loss in color. Bleachability in the fixing bath was also determined, but none of the above samples bleached under these conditions. Thiosulfate retention values were determined by the Ross-Crabtree Method on unexposed film coatings, processed in a commercial Recordak film processing machine.

Example 2.—1-[2-hydroxy-5-(2,4,4-trimethyl-2-pentyl)phenyl]-2,4,6-triphenylpyridinium iodide



The procedure for preparing the above compound was the same as Example 1 above, except that 2-amino-4-(2,4,4-trimethyl-2-pentyl)phenol was substituted for the m-aminophenol.

This compound was tested as a mordant in similar manner with the same dye as in Example 1 above. The results indicated that this compound is an effective "alkali-release" mordant and does not retain any dye or measurable thiosulfate ion residue, after complete processing.

Example 3.—1-(3,5-dibromo-4-hydroxyphenyl)-4,6-diphenyl-2-picolinium iodide



The above compound was prepared in accordance with the procedure of Example 1 above, except that the reactants were 2-methyl-4,6-diphenylpyrylium iodide and 4-amino-2,6-dibromophenol.

It was tested for mordanting ability, "alkali-release" properties and hypo retention in the same manner as that described in Example 1. The results showed good mordanting of the specified dye of Example 1, effective release and bleaching of the dye on development, and no measurable hypo retention from the fixing bath.

In place of the pyrylium compounds and the aminophenol compounds used in above Examples 1 to 3, there can be substituted an equivalent amount of any other of the intermediate compounds coming under Formulas IV and V above to give the corresponding compounds which likewise function effectively as "alkali-release" mordants in photographic layers. For example, other suitable pyrylium salt intermediates include 2-methyl-4,6-di-m (and p) tolylpyrylium halides, 2,6-dimethyl-4-(3-pyridyl)pyrylium halides, 2,4-diphenyl-6-propylpyrylium halides, 2-ethyl-4,6-di-p-tolylpyrylium halides, 2,4,6-triphenylpyrylium chloride, and the like, which are reacted with an aminophenol such as m-aminophenol, 2-amino-4-(2,4,4-trimethyl-2-pentyl)phenol, 4-amino-2,6-dibromophenol, etc., in accordance with the processes of the above examples.

The photographic elements prepared with the above-described mordants of the invention comprise a support material having thereon at least one hydrophilic colloid layer containing a mordant of the invention, which layer may also contain a light-sensitive silver halide. However, the preferred light-sensitive photographic elements comprise a support having thereon at least one hydrophilic colloid layer containing a mordant of the invention and at least one light-sensitive silver halide emulsion layer. The mordant containing light-screening and antihalation layers are customarily prepared by coating on the support or photographic element by methods well known in the art, a water solution comprising at least one mordant of the invention, an acid dye, a water-permeable hydrophilic colloid binder and a coating aid such as saponin. For most purposes, it is also desirable to add agents to harden the colloidal binder material so that the light-screening layer will remain intact in the photographic element during and following the processing operations. The pH of the coating solution is adjusted when necessary to a level that is compatible with the light-sensitive emulsion layer by the usual methods. The proportions of mordant, dye, colloidal binder, hardener and coating aid may be varied over wide ranges and will depend upon the specific re-

quirements of the photographic element being produced. The methods used to determine the optimum compositions are well known in the art and require no further elucidation here. Suitable support materials include any of those used in photography such as cellulose acetate, cellulose propionate, cellulose acetate-butyrate, cellulose nitrate, synthetic resins such as nylon, polyesters, polystyrene, polypropylene, etc., paper and the like.

Suitable hydrophilic colloid materials that can be used in the mordant containing compositions and layers, and photographic elements, of the invention include gelatin, albumin, collodion, gum arabic, agar-agar, cellulose derivatives such as alkyl esters of carboxylated cellulose, hydroxy ethyl cellulose, carboxy methyl hydroxy ethyl cellulose, synthetic resins, such as the amphoteric copolymers described by Clavier et al. in U.S. Patent 2,949,442, issued Aug. 16, 1960, polyvinyl alcohol, polyvinyl pyrrolidone, and others well known in the art. The above-mentioned amphoteric copolymers are made by polymerizing the monomer having the formula:



wherein R' represents an atom of hydrogen or a methyl group, and a salt of a compound having the general formula:



wherein R' has the above-mentioned meaning, such as an alkylamine salt. These monomers can further be polymerized with a third unsaturated monomer in an amount up to about 20 percent, and preferably from 5-15 percent of the total weight of monomer used, such as an ethylene monomer that is copolymerizable with the two principal monomers. The third monomer may contain either a basic group or an acid group and may, for example, be vinyl acetate, vinyl chloride, acrylonitrile, methacrylonitrile, styrene, acrylates, methacrylates, acrylamide, methacrylamide, etc. Examples of these polymeric gelatin substitutes are copolymers of allylamine and methacrylic acid; copolymers of allylamine, acrylic acid and acrylamide; hydrolyzed copolymers of allylamine, methacrylic acid and vinyl acetate; the copolymers of allylamine, acrylic acid and styrene; the copolymers of allylamine, methacrylic acid and acrylonitrile; etc.

The dyes that can be effectively mordanted in accordance with our invention include any filter dye that has one or more acidic group substituents such as sulfo or carboxyl groups, for example, the oxonol dyes described and claimed in copending application of Joseph Bailey, Canadian Patent 690,133 issued July 7, 1964, having the formula:



and more particularly the dyes of the formula:



wherein Z' represents the nonmetallic atoms necessary to complete a 1-carboxyalkyl-3-hydrocarbon substituted hexahydro-2,4,6-trioxo-5-pyrimidine nucleus, n' in each case is an integer of from 1 to 3, each R<sub>7</sub> represents a carboxyalkyl group in which the carboxy substituent is attached to an alkyl group having from 1 to 2 carbon atoms, R<sub>8</sub> is an alkyl group of from 1 to 8 carbon atoms or an aryl group such as phenyl or an alkyl or alkoxy substituted phenyl group, and X'' is hydrogen or an alkyl group of from 1 to 4 carbon atoms, such that no more than one X''

is an alkyl group. Other suitable acid dyes include the benzoxazolepyrazolone merocyanine dyes described in French Patent 1,359,682, issued Mar. 24, 1964, having the formula:



wherein  $\text{R}_9$  represents an alkyl group such as methyl, ethyl, propyl, isopropyl, butyl, isobutyl, tertiary butyl, etc., or a carboxyalkyl group, such as carboxymethyl, carboxyethyl, carboxypropyl, etc., or a sulfoalkyl group, such as sulfoethyl, sulfopropyl, sulfobutyl, etc.;  $\text{Z}''$  represents the nonmetallic atoms necessary to complete a heterocyclic nucleus of the benzoxazole series (including benzoxazole and benzoxazole substituted with substitutions such as methyl, ethyl, phenyl, methoxy, ethoxy, chlorine, bromine, etc.) or a nucleus of the benzoxazole series which has a sulfo-substituent on the benzene ring as well as one or more of the above-mentioned simple substituents, such that when  $\text{R}_9$  represents an alkyl group,  $\text{Z}''$  represents the sulfo-substituted benzoxazole nucleus and when  $\text{R}_9$  represents a carboxyalkyl group or a sulfo-alkyl group,  $\text{Z}''$  represents the nonmetallic atoms necessary to complete a benzoxazole nucleus;  $\text{Q}$  represents the nonmetallic atoms necessary to complete a heterocyclic nucleus of the sulfo-phenyl pyrazolinone series and  $n'$  is an integer from 1 to 3. However, the invention is not limited to just those dyes coming within the general formulas of the above-mentioned copending applications, since as previously set forth any filter dye containing one or more sulfo or carboxyl groups can be employed. For example, the yellow dyes mentioned in Mader et al. U.S. Patent 3,016,306, issued Jan. 9, 1962, columns 5 and 6.

Typical light-filtering dyes include, for example, bis(1-butyl - 3 - carboxymethylhexahydro - 2,4,6 - trioxo - 5 - pyrimidine)pentamethineoxonol, bis(1 - carboxymethyl - 3 - cyclohexylhexahydro - 2,4,6 - trioxo - 5 - pyrimidine)pentamethineoxonol, bis(1 - butyl - 3 - carboxymethylhexahydro - 2,4,6 - trioxo - 5 - pyrimidine)trimethineoxonol, bis(1 - carboxymethylhexahydro - 3 - octyl - 2,4,6 - trioxo - 5 - pyrimidine)methineoxonol, 4 - [(3 - ethyl - 2(3H) - benzoxazolylidene)ethylidene] - 3 - methyl - 1 - (p - sulfophenyl) - 2 - pyrazolin - 5 - one monosulfonated, 4 - [(3 - ethyl - 2 - (3H) - benzoxazolylidene) - 2 - butenylidene] - 3 - methyl - 1 - (p - sulfophenyl) - 2 - pyrazolin - 5 - one monosulfonated, 4 - [(3 -  $\beta$  - carboxyethyl - 2(3H) - benzoxazolylidene)ethylidene] - 3 - methyl - 1 - (p - sulfophenyl) - 2 - pyrazolin - 5 - one, 4 - [(3 -  $\beta$  - carboxyethyl - 2(3H) - benzoxazolylidene) - 2 - butenylidene] - 3 - methyl - 1 - (p - sulfophenyl) - 2 - pyrazolin - 5 - one, bis(1 butyl - 3 - carboxymethyl - 5 - barbituric acid)trimethine oxonol, bis(1 - butyl - 3 - carboxymethyl - 5 - barbituric acid)pentamethineoxonol, bis[3 - methyl - 1 - (p - sulfophenyl) - 2 - pyrazolin - 5 - one - (4) ]methineoxonol, bis[3 - methyl - 1 - (p - sulfophenyl) - 2 - pyrazolin - 5 - one - (4) ]trimethineoxonol, bis[3 - methyl - 1 - (p - sulfophenyl) - 2 - pyrazolin - 5 - one - (4) ]pentamethineoxonol, bis[3 - methyl - 1 - (p - sulfophenyl) - 5 - pyrazolone - (4) ]pentamethineoxonol, and typical ultraviolet absorbing dyes include the 2,5-bis(substituted sulfophenyl)thiazolo[5,4 - d]thiazole disodium salts of French Patent 1,359,924, issued Mar. 23, 1964, such as 2,5 - bis(o - methoxy - x - sulfophenyl)thiazolo[5,4 - d]thiazole disodium salt, 2,5 - bis(o - hexyloxy - x - sulfophenyl)thiazolo[5,4 - d]thiazole disodium salt, 2,5 - bis(o - decyloxy - x - sulfophenyl)thiazolo[5,4 - d]thiazole disodium salt, 2,5 - bis(o - methyl - x - sulfophenyl)thiazolo[5,4 - d]thiazole disodium salt, 2,5 - bis(p - propyl - x - sulfophenyl)thiazolo[5,4 - d]thiazole disodium salt, etc.; the ultraviolet absorbing dyes of Sawdey U.S. Patent 2,739,888, issued Mar. 27, 1956, such as 3 - phenyl - 2 - phenylimino - 5 - o - sulfobenzal - 4 -

thiazolidone sodium salt, 5 - (4 - methoxy - 3 - sulfobenzal) - 3 - phenyl - 2 - phenylimino - 4 - thiazolidone (sodium salt), 3 - phenyl - 2 - phenylimino - 5 - [3 - (3 - sulfobenzamido) - benzal] - 4 - thiazolidone (sodium salt), 3 - benzyl - 2 - phenylimino - 5 - o - sulfobenzal - 4 - thiazolidone (sodium salt), 5 - (2,4 - dicarboxymethoxybenzal) - 3 - phenyl - 2 - phenylimino - 4 - thiazolidone sodium salt, etc., tartrazine, and the like filter dyes.

Hardening materials that may be used to advantage include such hardening agents as formaldehyde; a halogen-substituted aliphatic acid such as mucobromic acid as described in White U.S. Patent 2,080,019, issued May 11, 1937; a compound having a plurality of acid anhydride groups such as 7,8 - diphenylbicyclo(2,2,2) - 7 - octene-2,3,5,6 - tetra - carboxylic dianhydride, or a dicarboxylic or a disulfonic acid chloride such as terephthaloyl chloride or naphthalene-1,5-disulfonyl chloride as described in Allen and Carroll U.S. Patents 2,725,294 and 2,725,295, both issued Nov. 29, 1955; a cyclic 1,2-diketone such as cyclopentane-1,2-dione as described in Allen and Byers U.S. Patent 2,725,305, issued Nov. 29, 1955; a bisester of methanesulfonic acid such as 1,2-di(methanesulfonyloxy)ethane as described in Allen and Laakso U.S. Patent 2,726,162, issued Dec. 6, 1955; 1,3-dihydroxy-methylbenzimidazol-2-one as described in July, Knott and Pollak, U.S. Patent 2,732,316, issued Jan. 24, 1956; a dialdehyde or a sodium bisulfite derivative thereof, the aldehyde groups of which are separated by 2-3 carbon atoms, such as  $\beta$ -methyl glutaraldehyde bis-sodium bisulfite as described in Allen and Burness, Canadian Patent No. 588,451, issued Dec. 8, 1959; a bis-aziridine carboxamide such as trimethylene bis (1-aziridine carboxamide) as described in Allen and Webster U.S. Patent 2,950,197, issued Aug. 23, 1960; or 2,3-dihydroxydioxane as described in Jeffreys U.S. Patent 2,870,013, issued Jan. 20, 1959.

The photographic element utilizing our light-screening layers have light-sensitive emulsion layers containing silver chloride, silver bromide, silver chlorobromide, silver iodide, silver bromoiodide, silver chlorobromoiodide, etc., as the light-sensitive material. Any light-sensitive silver halide emulsion layers may be used in these photographic elements. The silver halide emulsion may be sensitized by any of the sensitizers commonly used to produce the desired sensitometric characteristics.

In the accompanying drawing which further illustrates the preferred photographic elements of our invention:

FIG. 1 shows light-screening layer 10 comprising gelatin, an acid substituted filter dye and the mordant of Example 1 coated over a light-sensitive silver halide emulsion layer 11 which is coated on support 12.

FIG. 2 shows antihalation layer 15 comprising gelatin, an acid substituted dye and the mordant of Example 1 coated adjacent to support 16 and a light-sensitive silver halide emulsion layer 14 coated over layer 15.

FIG. 3 shows a multilayer color element comprising a support 21 having a red-sensitive silver halide emulsion layer 20 coated thereon, a green-sensitive silver halide emulsion layer 19 coated over layer 20, a light-sensitive layer 18 comprising gelatin, an acid substituted dye, and the mordant of Example 1 coated over layer 19, and a blue-sensitive silver halide emulsion layer 17 coated over layer 18.

Additional typical mordants of Formulas I and II used to advantage according to our invention are as follows:

| Example: | Mordant                                                                                                        |
|----------|----------------------------------------------------------------------------------------------------------------|
| 4 -----  | 1 - dodecyl - 2,6 - diphenyl - 4 - (4 - hydroxyphenyl)pyridinium iodide.                                       |
| 5 -----  | 3 - dodecyl - 6 - hydroxy - 2 - styrylbenzothiazolium iodide.                                                  |
| 6 -----  | 3 - benzyl - 1 - ethyl - 2 - [4 - (4' - hydroxy - $\alpha$ - naphthyl)butadienyl - 1,4]benzimidazolium iodide. |
| 7 -----  | 3 - ethyl - 2 - [6 - (4 - hydroxyphenyl) -                                                                     |

Example:

- Mordant  
hexatrienyl - 1,3,5] -  $\beta,\beta$  - naphthoxazolum iodide.
- 8 ----- N-octadecyl - N - (4 - hydroxy- $\alpha$ -naphthyl)pyrrolidinium iodide.
- 9 ----- N,N,N - tridodecyl - N - (2 - hydroxyphenyl)ammonium chloride.
- 10 ----- N,N - diphenyl - N - (2 - hydroxyphenyl) - N - decylammonium iodide.
- 11 ----- N - benzyl - N,N - didodecyl - N - (4 - hydroxyphenyl)ammonium iodide.

The mordants 4 through 11 are substituted for 1-m-hydroxyphenyl-2,4,6-triphenylpyridinium iodide in Example 1 and are found to be excellent mordants which completely release acid dyes mordanted with them upon treatment with alkaline processing solutions. Mordants 4 through 8 are produced by the methods described previously herein. Mordants 9 through 11 are produced by alkylating the amine by methods well known in the art.

The use of our "alkali-release" mordants in light-screening layers over light-sensitive silver halide emulsion layers, and in antihalation undercoat layers, to produce improved photographic elements has been illustrated in the preceding examples. However, it will be apparent that the mordants of the invention can also be advantageously used in light-screening layers between two or more color sensitized silver halide emulsion layers, or in antihalation backing layers, or incorporated directly in light-sensitive silver halide emulsion layers, or they can be used to prepare imbibition dye transfer blanks of improved properties.

The invention has been described in detail with particular reference to preferred embodiments thereof but it will be understood that variations and modifications can be effected within the spirit and scope of the invention as described hereinabove and as defined in the appended claims.

We claim:

1. A photographic element comprising a support material having thereon a hydrophilic colloid layer containing at least one compound selected from those represented by the formula:



and



wherein  $m$  and  $n$  each represent an integer of from 1 to 2, R represents a member selected from the class consisting of the hydrogen atom, an alkyl group, and an aryl group,  $R_1$  represents a member selected from the class consisting of an alkyl group, and an aryl group,  $R_2$  and  $R_3$  each represents a member selected from the class consisting of an alkyl group, and an aryl group,  $R_2$  and  $R_3$  together represent a divalent alkylene group of from 4 to 5 carbon atoms in the chain, X represents an acid anion, B represents a member selected from the class consisting of the group  $CH=CH$ , the group  $(CH=CH)_2$ , the group  $(CH=CH)_3$ , and the p-phenylene group, and Z represents the nonmetallic atoms necessary to complete a 5 to 6 membered heterocyclic nucleus selected from the class consisting of a thiazole nucleus, a benzothiazole nucleus, a naphthothiazole nucleus, a thionaphtheno-7',6',4,5-thiazole nucleus, an oxazole nucleus, a benzoxazole nucleus, a naphthoxazole nucleus, a selenazole nucleus, a benzoselenazole nucleus, a naphthoselenazole nucleus, a thiazoline nucleus, a quinoline nucleus, an isoquinoline nucleus, a 3,3-dialkylindolenine nucleus, a pyridine nucleus, an imidazole nucleus, a benzimidazole nucleus, a naphthimidazole nucleus, a thiadiazole nucleus, an oxadiazole nucleus, a triazole nucleus and a tetrazole nucleus,

provided that at least one of said R, said  $R_1$  and Z contains a phenolic group, and wherein said compound has a molecular weight of at least 300, said element containing light-sensitive silver halide.

2. A light-sensitive photographic element comprising a support material having thereon a hydrophilic colloid layer containing at least one substantially non-diffusible salt of a water-soluble acid dye with a mordant compound of the formula:



- 15 wherein  $j$  represents an integer of from 1 to 3,  $d$  represents an integer of from 1 to 2,  $R_4$  and  $R_6$  each represents a member selected from the class consisting of the hydrogen atom, a halogen atom, an alkyl group, an aryl group, an alkoxy group, an aryloxy group, a 2-thienyl group, a 2-pyrryl group, a 2-indolyl group, a 3-indolyl group, a 2-furyl group, a 3-pyridyl group, and a 4-pyridyl group, and X represents an acid anion, said compound having a molecular weight of at least 300, said element containing light-sensitive silver halide.

- 20 25 3. A light-sensitive photographic element comprising a support material having thereon at least two hydrophilic colloid layers, at least one of said hydrophilic colloid layers being a light-sensitive silver halide emulsion layer and at least one of said hydrophilic layers containing at least one nondiffusible salt of a water-soluble acid dye with a compound of the formula:



- 35 wherein  $j$  represents an integer of from 1 to 3,  $d$  represents an integer of from 1 to 2,  $R_4$  and  $R_6$  each represents a member selected from the class consisting of the hydrogen atom, a halogen atom, an alkyl group, aryl group, an alkoxy group, an aryloxy group, a 2-thienyl group, a 2-pyrryl group, a 2-indolyl group, a 3-indolyl group, a 2-furyl group, a 3-pyridyl group, and a 4-pyridyl group, and X represents an acid anion, said compound having a molecular weight of at least 300.

- 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245

## 15

compound is 1-(3,5-dibromo-4-hydroxyphenyl)-4,6-diphenylpicolinium iodide.

9. A photographic element of claim 2 wherein said acid dye is bis[3-methyl-p-sulfophenyl-2-pyrazolin-5-one-(4)]-pentamethineoxonol and said compound is 1-m-hydroxyphenyl-2,4,6-triphenylpyridinium iodide.

10. A light-sensitive photographic element according to claim 2 wherein at least one of said dye components of said salts is a dye selected from the group consisting of 4-[(3-ethyl-2(3H)-benzoxazolylidene)ethylidene]-3-methyl-1-p-sulfophenyl-2-pyrazolin-5-one monosulfonated, bis(1-butyl-3-carboxymethyl-5-barbituric acid)trimethineoxonol, 4-[4-(3-ethyl-2(3H)-benzoxazolylidene)-2-butenyldene]-3-methyl-1-p-sulfophenyl-2-pyrazolin-5-one monosulfonated, bis(1-butyl-3-carboxymethyl-5-barbituric acid)pentamethineoxonol, bis[3-methyl-1-(p-sulfophenyl)-2-pyrazolin-5-one-(4)]methineoxonol, bis[3-methyl-1-(p-sulfophenyl)-2-pyrazolin-5-one-(4)]trimethineoxonol and bis[3-methyl-1-(p-sulfophenyl)-2-pyrazolin-5-one-(4)]pentamethineoxonol.

11. A light-sensitive photographic element according to claim 2 wherein at least one of said dye components of said salts is a dye selected from the group consisting of 4-[(3-ethyl-2(3H)-benzoxazolylidene)ethylidene]-3-methyl-1-p-sulfophenyl-2-pyrazolin-5-one monosulfonated, bis(1-butyl-3-carboxymethyl-5-barbituric acid)trimethineoxonol, 4-[4-(3-ethyl-2(3H)-benzoxazolylidene)-2-butenyldene]-3-methyl-1-p-sulfophenyl-2-pyrazolin-5-one monosulfonated, bis(1-butyl-3-carboxymethyl-5-barbituric acid)pentamethineoxonol, bis[3-methyl-1-(p-sulfophenyl)-2-pyrazolin-5-one-(4)]methineoxonol, bis[3-methyl-1-(p-sulfophenyl)-2-pyrazolin-5-one-(4)]trimethineoxonol and bis[3-methyl-1-(p-sulfophenyl)-2-pyrazolin-5-one-(4)]pentamethineoxonol, and wherein the said hydrophilic colloid layer comprises gelatin.

12. An element comprising a support material having thereon a hydrophilic colloid layer containing a salt of a

## 16

water-soluble acid dye and at least one compound selected from those represented by the formula:



5 and



10 wherein  $m$  and  $n$  each represent an integer of from 1 to 2, R represents a member selected from the class consisting of the hydrogen atom, an alkyl group, and an aryl group,  $R_1$  represents a member selected from the class 15 consisting of an alkyl group, and an aryl group,  $R_2$  and  $R_3$  each represents a member selected from the class consisting of an alkyl group, and an aryl group,  $R_2$  and  $R_3$  together represent a divalent alkylene group of from 4 to 5 carbon atoms in the chain, X represents an acid anion, B 20 represents a member selected from the class consisting of the group  $CH=CH$ , the group  $(CH=CH)_2$ , the group  $(CH=CH)_3$ , and the p-phenylene group, and Z represents the nonmetallic atoms necessary to complete a heterocyclic nucleus having from 5- to 6-members in the heterocyclic ring, provided that at least one of the said R, 25 said  $R_1$ , and said Z groups contains a phenolic group, and wherein said compound has a molecular weight of at least 300.

## References Cited

## UNITED STATES PATENTS

3,016,306 1/1962 Mader et al. ----- 96-84 XR  
3,271,148 9/1966 Whitmore ----- 96-84 XR

35 NORMAN G. TORCHIN, Primary Examiner.

R. SMITH, Assistant Examiner.

U.S. CL. X.R.

96-057, 029; 117-167

UNITED STATES PATENT OFFICE  
**CERTIFICATE OF CORRECTION**

Patent No. 3,425,833

February 4, 1969

Robert C. Taber et al.

It is certified that error appears in the above identified patent and that said Letters Patent are hereby corrected as shown below:

Column 14, lines 32 to 37, the formula should appear as shown below:



same column 14, lines 70 and 71, "1-(3,5-dibromo-4-hydroxy-phenyl-4,6-di-ium iodide" should read -- 1-m-hydroxyphenyl-2,4,6-triphenylpyridinium iodide --. Column 16, lines 3 to 6, that part of the formula reading

$$-\overset{\mid}{N}(=CH-)$$

should read

$$\begin{array}{c} | \\ -N(=CH-) \\ | \\ X \end{array}$$

Signed and sealed this 5th day of May 1970.

(SEAL)  
Attest:

EDWARD M. FLETCHER, JR.  
Attesting Officer

WILLIAM E. SCHUYLER, JR.  
Commissioner of Patents